

H. JANDER.

APPARATUS FOR THE RECOVERY OF ARSENIOUS AND SELENIOUS OXIDS.

APPLICATION FILED APR. 3, 1919.

1,321,211.

Patented Nov. 11, 1919.

2 SHEETS—SHEET 1.



H. JANDER.

APPARATUS FOR THE RECOVERY OF ARSENIOUS AND SELENIOUS OXIDS.

APPLICATION FILED APR. 3, 1919.

1,321,211.

Patented Nov. 11, 1919.

2 SHEETS—SHEET 2.



Inventor  
Henry Jander  
By Maurice, Block  
attorney.

# UNITED STATES PATENT OFFICE.

HENRY JANDER, OF BROOKLYN, NEW YORK.

## APPARATUS FOR THE RECOVERY OF ARSENIOUS AND SELENIOUS OXIDS.

1,321,211.

Specification of Letters Patent. Patented Nov. 11, 1919.

Application filed April 3, 1919. Serial No. 287,262.

To all whom it may concern:

Be it known that I, HENRY JANDER, a citizen of the United States of America, residing at Brooklyn, Kings county, State of New York, have invented certain new and useful Improvements in Apparatus for the Recovery of Arsenious and Selenious Oxids, of which the following is a full, clear, and exact description.

10. This invention relates to an apparatus for carrying out the process for the recovery of selenious and arsenious oxids as a by-product resulting from the burning of a pyrite. Sulfur, selenium and arsenic are relative elements and are always found associated in a more or less degree; they are combustible and form oxids when burned in free oxygen, to wit:



20. Owing to the difference in their atomic weight, they form gases of different specific gravities. It is in the form of oxids where selenium, arsenic and sulfur commence to diverge. When the burner gases from the pyrite are led into a chamber and allowed to cool, to about 200 degrees C., the arsenious oxid crystallizes and precipitates in the form of a fine dust. If these gases are 30 cooled to a somewhat lower degree, selenious oxid will be precipitated, but the sulfurous oxid being a more stable gas, under ordinary atmospheric pressure and temperature, will remain floating in the chamber. 35 If this gaseous sulfurous oxid is carefully drawn from the chamber and led into a flask containing hot water mixed with nitric acid, the following reaction will take place:



40. When drawing the sulfurous gases off care must be taken not to agitate the selenious and arsenious oxids, or they will become mixed with the sulfurous gases, thereby contaminating them. If the foregoing experiments are carefully carried out and the drawn off gases are submitted to distillation, pure sulfuric acid will result and oxid of arsenic and selenium will be recovered as 45 by-products.

To carry out the operations above described, said operations being an epitomized recitation of my improved process, I have designed a special apparatus to carry out 50 the steps of the process.

In the accompanying drawings, which form a part of this specification,

Figure 1 is a sectional view of a refrigerating apparatus within which the burner gases from the pyrite burner are cooled 60 down to produce the results described; and

Fig. 2 is a similar view of an oven or muffle within which the sulfur dioxide, which has been liberated in the refrigerator, is reheated and then mixed with nitric acid 65 fumes.

The apparatus herein illustrated consists of a suitable housing 3 containing cooling or refrigerating cells 4, 5, 6, 7 and 8, and a pyrite burner 9 of any suitable construction. 70 The pyrite burner 9 is connected to cell 4 by a passage 10. Cell 4 is connected to cell 5 by a passage 11, said passage being located adjacent the upper end of said cells. Cells 5 and 6 are connected by passage 12 near the 75 bottoms thereof, cells 6 and 7 and cells 7 and 8 being likewise connected, by passages 13 and 14, respectively.

A further element of the apparatus consists of a reheating oven 16 having a main 80 flue 17 surrounded by smaller flues or tubes 18 placed in communication with a fire-box 19 and a chimney 20. The main flue 17 is connected by a passage 21 with a chamber 22 containing a pot or container 23 for diluted nitric acid. The chamber 22 is connected by passages 24 and 25 with a Glover tower (which is not shown). The re heater 16 may be of any desirable construction embodying the elements above described; 85 hence a detailed description of the herein illustrated re heater will be omitted. 90

The method of recovering selenious and arsenious oxids will now be explained. Pyrites will be placed in burner 9 and transformed into gases by the application of heat. The gases thus generated will pass through duct or passage 10 into the lower portion 100 of the cooling cell 4 which contains cooling coils 27 through which brine is forced. The gases as they rise and pass through the coils will be cooled to about five hundred and thirty degrees centigrade. The gases will now pass through passage 11 into cell 5, thence down through the cooling pipes 105 28, which also contain brine, into the lower chamber 29, thence into the lower chamber of cell 6 up through cooling pipes 30, where their temperature will be reduced to about 200° C. This cooling action will cause the 110

precipitation of the arsenious oxid in the form of dust which will settle on the bottom of the chamber. The unprecipitated gases will pass through passage 13 into cell 7, thence downward through cooling coils 31, containing brine, into lower chamber 32 of cell 7; thence through passage 14 into cell 8, thence upward through cooling coils 33. When the gases have reached this point they will have been cooled to about one hundred and fifty degrees C. causing the precipitation of selenious oxid. The remaining gas, sulfurous oxid, will flow into duct or passage 15, thence into the main flue 17 of the re-heater 16. The sulfurous oxid ( $\text{SO}_2$ ) contained in duct 17, will be reheated by the hot gases in the circulating flues 18 which emanate from the fire on the grate in the fire-box 19. The reheated  $\text{SO}_2$  will pass through the passage 21 into chamber 22 containing pot 23, which in turn is charged with a solution of water, and nitric acid, the fumes of which will mix with the  $\text{SO}_2$ . The following reaction will now take place:

25  $3\text{SO}_2 + 2\text{HNO}_3 + 2\text{H}_2\text{O} = 3\text{H}_2\text{SO}_4 + \text{N}_2\text{O}_2$ ;

or in other words, three volumes of sulfur dioxid plus two volumes of nitric acid plus two volumes of water=three volumes sulfuric acid gas plus nitrous oxid. These resulting gases pass through passages 24 and 25 into a Glover tower (not shown), after which they will be subjected to the usual process for producing sulfuric acid.

30 35 It would be noted that while the  $\text{SO}_2$  is passing through the re-heater it never comes

in contact with the gases of combustion. My improved process is intended for the recovery of arsenious and selenious oxids as a byproduct in the manufacture of sulfuric acid.

Having described my invention, what I claim is:

1. In an apparatus for the recovery of arsenic and selenium the combination of a 45 pyrite burner, a plurality of cells adjacent thereto, cooling means in each cell, and a reheating device connected with one of the cells.

2. In an apparatus for the recovery of 50 arsenic and selenium, a pyrite burner, a refrigerating device and a reheating device consisting of a main flue, means to cause hot gases to circulate around said flue exteriorly thereof, a chamber in communication with 55 the main flue, and means to contain an acid located in said chamber.

3. In an apparatus for the recovery of arsenic and selenium, a plurality of intercommunicating chambers, coils located 60 within and intermediate the top and bottom of each chamber adapted for the passage therethrough of a refrigerant, and a reheating device connected with one of the chambers.

Signed at New York city, N. Y., this 1st day of April, 1919.

HENRY JANDER.

Witnesses:

EDWARD A. JARVIS,  
MAURICE BLOCK.